# EUROPEAN PATENT SPECIFICATION

(11) **EP 3 627 525 B1**
(45) Date of publication and mention of the grant of the patent: **03.03.2021**
(21) Application number: 19190437.4
(22) Date of filing: 07.08.2019
(51) Int. Cl.: H01F 41/02

(54) **A METHOD FOR IMPROVING PERFORMANCE OF SINTERED NDFEB MAGNET**
VERFAHREN ZUR VERBESSERUNG DER LEISTUNG EINES GESINTERTEN NDFEB-MAGNETEN
PROCÉDÉ PERMETTANT D'AMÉLIORER LA PERFORMANCE D'UN AIMANT NDFEB FRITTÉ

(30) Priority: 16.08.2018 CN 201810932329
(43) Date of publication of application: 25.03.2020
(73) Proprietor: Yantai Shougang Magnetic Materials Inc., 265500 Yantai (CN)
(72) Inventor: Chen, Xiulei, Yantai, 265500 (CN); Peng, Zhongjie, Yantai, 265500 (CN); Liu, Guangyang, Yantai, 265500 (CN); Zhu, Xiaonan, Yantai, 265500 (CN)
(74) Representative: Gulde & Partner

(56) References cited:
- CN-A- 103 920 879
- US-A1- 2002 115 390
- US-A1- 2004 045 637
- US-A1- 2013 043 218

## Description

### BACKGROUND OF THE INVENTION

### 1. Field of the Invention

The present invention relates generally to a method for improving performance of sintered NdFeB magnet.

### 2. Description of the Prior Art

For the large size NdFeB magnet, component segregation is easy to occur during the sintering and annealing process. This phenomenon is attributed to rare earth volatilization and capillary tension during liquid phase sintering process. This will result in a different elemental distribution at different locations of the blank, especially rare earth elements causing a difference in magnetic properties at different locations of the same blank. This situation will become more serious if the single blank size is larger or the grain size is smaller.

In addition, the traditional NdFeB products are generally processed into finished products by mechanical machining after sintering and annealing. The machining methods involve cutting, grinding, drilling, chamfering, etc. The machining technology is relatively mature and easy to operate and also has high machining efficiency and high machining precision. However, during the machining of the annealed blank, surface stress is generated on the surface of the product, causing damage to the surface crystal structure, and then resulting in attenuation of magnetic properties, which degrades the performance of the magnet from the blank. For products with large specific surface area and irregular shape product, the magnetic attenuation caused by the machining is more serious. At the same time coolant is used in the machining process for lowering the temperature. Research shows that the cutting fluid can erode to a depth of several micrometers in the magnet, which will affect the magnetic properties and corrosion resistance.

Chinese patent CN105741994B provides a method for directly machining a neodymium iron boron green compact into a finished product shape before sintering, thereby avoiding damage to the performance of the magnet during machining and maintaining the performance state of the magnet after heat treatment. Further examples may be found in US 2004/0045637 A1. However, there are some shortcomings in the method of completely machining the green compact into a finished product before sintering. Machining the green compact by using conventional equipment and methods has great problems in operability and precision, because the density of the green compact is too low compared with the sintered blank. The green compact is easy to be damaged while machining and the pass rate is reduced. To ensure that each machining step is carried out in an inert gas atmosphere or protective oil, the equipment requirements are strict and the costs are increased. Furthermore, it is difficult to process the green compact directly into finished products if the product size is too small, and the precision will be poor. For some products with curved profile or irregular shape, the sintering shrinkage rate in different directions is difficult to calculate accurately, which may cause a large deviation from the target product size. In addition, machining the green compact directly into product size before sintering will increase the surface area, which will cause easier nitride forming or oxidation while sintering, which may reduce the magnetic performance of the magnet.

### SUMMARY OF THE INVENTION

According to one aspect of the invention there is provided a method of preparing a sintered NdFeB magnet as defined in claim 1. The method comprises the steps of:
a) pressing magnetic powders into a green compacts under a magnetic field and then demagnetization;
b) isostatic pressing the green compact;
c) fixing the green compact on a special device as defined below, and then machining the green compact into a finished shape and corresponding size on one or two surfaces among an orientation surface, non-orientation surface and pressing surface;
d) sintering and annealing the the machined green compact; and
e) machining the obtained blank into a finished product.

According to one embodiment, in step b) of isostatic pressing the pressure is between 150MPa to 400MPa.

According to another embodiment, the density of green compact after isostatic pressing is between 4.5-5.5g/cm³.

According to another embodiment, in step c) the orientation surface refers to the surface parallel to the orientation magnetic field and not in contact with an indenter during the pressing process;
the pressing surface refers to the plane in contact with the indenter during the pressing process;
the non-orientation surface refers to the plane perpendicular to the orientation surface and the pressing surface; and
the corresponding size of the finished product refers to the size of the finished product multiplied by the shrinkage rate of the sintering process.

According to another embodiment, step c) of machining the machining green compact is operated in the atmosphere of nitrogen or rare gas.

According to another embodiment, step d) of sintering and annealing is performed under vacuum of below 5×1⁻¹Pa, a sintering temperature between 980°C to 1040°C, and an annealing temperature between 480°C to 600°C.

According to another embodiment, step e) of machining the blank refers to porcessing surfaces that have not been processed in step c) of machining the green compact.

According to the invention, a special device for machining a NdFeB green compact is provided. The special device comprises a reciprocating cutting mechanism, a cutting tooling, a green compact fixed tooling and a reciprocating lifting mechanism. The reciprocating cutting mechanism is connected to the cutting tooling and the reciprocating lifting mechanism is connected to the green compact fixed tooling.

The reciprocating cutting mechanism is adapted for reciprocating in a horizontal direction and the reciprocating lifting mechanism is adapted for realizing a reciprocating lifting in a vertical direction.

The green compact fixed tooling comprises a pair of trunking plates, a pair of limit guiding plates, guiding pins, adjusting bolts and a base. The pair of trunking plates is mounted on opposite sides of the base. The pair of limit guiding plates is mounted to the end of the trunking plates and the limit guiding plates are provided with the guiding pins and adjusting bolts.

The cutting tooling comprises a pair of wire fixing boards, cutting wires, adjusting screws, and a fixing plate. The pair of wire fixing boards is mounted on the fixing plate and the cutting wires are tensioned by means of the adjusting screws between the the pair of wire fixing boards.

In other words, the present disclosure provides a method including a step of machining the green compact into a finished shape and corresponding size on one or two surface among the orientation surface, non-orientation surface and pressing surface. And then normal sintering and annealing processes are performed, and the obtained magnet is processed into a finished product by conventional machining methods.

The invention provides for a special device contains four parts as: a reciprocating cutting mechanism (A), a cutting tooling (B), green compact fixed tooling (C) and the reciprocating lifting mechanism (D).

Using the method, the performance of sintered NdFeB magnet could be improved.

(Not falling under the protection scope of the present invention) The special device for machining NdFeB green compacts enhances machining precision and efficiency.

Using this method and the special device can reduce the variation of the composition and magnetic properties of the sintered magnet, reduce the loss of magnetic properties caused by the traditional machining process. At the same time, a damage to the green compact during the machining may be reduced. Further, the proportion of non-recyclable waste powders may be reduced. The comprehensive utilization rate of magnetic powder may be significantly improved.

### BRIEF DESCRIPTION OF THE DRAWINGS

Other advantages of the present invention will be readily appreciated, as the same becomes better understood by reference to the following detailed description, when considered in connection with the accompanying drawings, wherein:
Figure 1 is a schematic view of the overall structure of the special device according to an example of the present invention, and
Figure 2 is a schematic view showing the structure of the green compact fixed tooling in the special device according to an example of the present invention, and
Figure 3 is a schematic view showing the structure of the cutting tooling in the special device according to an example of the present invention.

### DESCRIPTION OF THE ENABLING EMBODIMENT

Referring to the Figures, the present invention will be described in an exemplary embodiment. The inventive preparation method may improve the performance of sintered NdFeB magnets. The exemplary method includes a first step of pressing the magnetic powders into green compact under a magnetic field and then demagnetization.

The method also includes a step of applying isostatic pressing to the green compact. The pressure of isostatic is between 150MPa to 400MPa, the density of green compact after isostatic is between 4.5-5.5g/cm³.

The method further includes step of fixing the green compact on a special device, and then machining the green compact into finished shape and corresponding size on one or two surface among the orientation surface, non-orientation surface and pressing surface. The orientation surface refers to the surface parallel to the orientation magnetic field and not in contact with the indenter during the pressing process; the pressing surface refers to the plane in contact with the press head during the pressing process; the non-orientation surface refers to the plane perpendicular to the orientation surface and the pressing surface; the corresponding size of the finished product refers to the size of the finished product multiplied by the shrinkage rate of the sintering process.

The method further includes steps of sintering and annealing the processed green compacts by conventional process. Sintering and annealing process are performed while the vacuum degree is below 5×10⁻¹ Pa, and the sintering temperature is between 980°C to 1040°C, the annealing temperature is between 480°C to 600°C.Then machining the magnet into finished products by traditional machining methods. The conventional machining is just executed on the surface that has not been processed in the green state.

The special device - as shown in Figure 1 through 3 - contains four parts as: a reciprocating cutting mechanism A, a cutting tooling B, the green compact fixed tooling C and the reciprocating lifting mechanism D.

The reciprocating cutting mechanism A is connected to the cutting tooling B, the reciprocating lifting mechanism D is connected to the green compact fixed tooling C, the green compact fixed tooling C and the cutting tooling B are Correspondingly; the reciprocating cutting mechanism A reciprocates in a horizontal direction, and the reciprocating lifting mechanism D realizes reciprocating lifting in a vertical direction. The green compact fixed tooling C is made up of a trunking plate 1, the limit guiding plate 2, the guiding pin 3, the adjusting bolt 4 and the base 5. The base 5 is correspondingly provided with two trunking plates 1 . At the end of the trunking plate 1 is provided with a limit guiding plate 2, the limit guiding plate 2 is provided with a guiding pin 3 and an adjusting bolt 4.The cutting tooling B is composed of a wire fixing board 6, a cutting wire 7, an adjusting screw 8, and a fixing plate 9, wherein the wire fixing board 6 is provided with a cutting wire 7. And the wire fixing board 6 is connected with the fixing plate 9. An adjusting screw 8 is arranged on the the wire fixing board 6.

To have a better understanding of the present invention, the examples set forth below provide illustrations of the present invention. The examples are only used to illustrate the present invention and do not limit the scope of the present invention.

### IMPLEMENTING EXAMPLE 1

The target size of product is: 10.0 mm (non-orientation surface) * 6.5 mm (orientation surface) * 8.0 mm (pressing surface), and the non-orientation surface is processed into a corresponding size of the finished product by using the special device of the present invention in the green state. The orientation surface and pressing surface are processed after annealing. Specific steps are as follows:
The magnetic powder with an average particle size of X50=4.0 µm was pressed into a green compact under 2.0T magnetic field, and then pressed by isostatic pressing at 150 MPa. The density of green compact after isostatic pressing was about 4.5 g/cm³, and the green compact size was 79.3 mm (Non-orientation surface) *38.2mm (orientation surface) * 44.8mm (pressing surface). Green compact weights 610.7g. The magnetic powder composition is PrNd 31.10 wt.%, Dy 1.50 wt.%, B 0.95 wt.%, Co 1.05 wt.%, Al 0.51 wt.%, Cu 0.15 wt.%, Ga 0.12 wt.%, Ti 0.11 wt.% .The balance is Fe and inevitable impurity elements. The green compact was placed on the base of the green compact fixed tooling, the wire groove plate with the groove width of 11.3 mm was selected, and the green compact was fastened by adjusting the bolt. A limit baffle with a slot spacing of 11.3mm is selected on the cutting tooling, and the diameter of the cutting wire used is 0.3mm. Start cutting the green compact along the non-orientation surface after the device is assembled. Each green compact is cut into 7 pieces with size of 11.0mm (non-orientation surface)*38.2mm (orientation surface)*44.8mm (pressing surface). The above operation was carried out in a nitrogen atmosphere. The magnetic powder produced by the cutting process can be simply collected and then subjected to secondary molding. The cut blank is sintered in a vacuum furnace. The sintering temperature was 980°C, and the temperature was kept for 10 hours. And then the sintered blank was annealed. The first-stage annealing temperature is 800°C, the temperature is kept for 3 hours, the second-stage aging temperature is 480°C, and the temperature is kept for 3 hours. The degree of vacuum during sintering and annealing was less than 5×10⁻¹ Pa. The annealing finished blank is subjected to conventional machining, the orientation surface and the pressing surface are polished after a wire cutting process, and the non-orientation surface only needs to be simply polished. Each green compact finally obtained 140 pieces of finished products having a size of 10.0 mm * 6.5 mm * 8.0 mm. During the green compact machining process, each isostatic green compact produces 13.8 g of magnetic powder, which can be directly pressed into a green compact after simple recycling. 50.5g of hard-to-recycle waste powder is produced during the sintering process and annealing process and traditional machining process. Total weight of the finished product is 546.0g, and the comprehensive utilization rate of the magnetic powder is 91.7%. Twenty pieces of products are selected randomly for analyzing. Total rare earth element content (TRE) and magnetic properties are listed in table 1.

**Table 1: TRE and magnetic properties distribution of example 1**

| sample | TRE(wt.%) | Br(T) | Hcj(kA/m) | Hk/Hcj | O(ppm) | N (ppm) |
|---|---|---|---|---|---|---|
| 1 | 30.97 | 1.323 (13.23 kGs) | 1767.12 (22.2 kOe) | 0.97 | 692 | 384 |
| 2 | 31.20 | 1.316 (13.16 kGs) | 1791.00 (22.5 kOe) | 0.98 | 686 | 365 |
| 3 | 30.98 | 1.322 (13.22 kGs) | 1767.12 (22.2 kOe) | 0.98 | 688 | 364 |
| 4 | 31.02 | 1.320 (13.20 kGs) | 1783.04 (22.4 kOe) | 0.98 | 677 | 365 |
| 5 | 31.03 | 1.321 (13.21 kGs) | 1775.08 (22.3 kOe) | 0.99 | 705 | 354 |
| 6 | 31.20 | 1.316 (13.16 kGs) | 1783.04 (22.4 kOe) | 0.98 | 685 | 397 |
| 7 | 31.18 | 1.317 (13.17 kGs) | 1783.04 (22.4 kOe) | 0.97 | 654 | 368 |
| 8 | 31.20 | 1.318 (13.18 kGs) | 1791.00 (22.5 kOe) | 0.96 | 687 | 384 |
| 9 | 31.15 | 1.320 (13.20 kGs) | 1775.08 (22.3 kOe) | 0.95 | 692 | 389 |
| 10 | 31.16 | 1.321 (13.21 kGs) | 1775.08 (22.3 kOe) | 0.98 | 657 | 401 |
| 11 | 31.16 | 1.320 (13.20 kGs) | 1775.08 (22.3 kOe) | 0.97 | 659 | 412 |
| 12 | 30.98 | 1.321 (13.21 kGs) | 1767.12 (22.2 kOe) | 0.96 | 687 | 378 |
| 13 | 30.97 | 1.323 (13.23 kGs) | 1767.12 (22.2 kOe) | 0.97 | 668 | 365 |
| 14 | 31.00 | 1.320 (13.20 kGs) | 1767.12 (22.2 kOe) | 0.98 | 649 | 396 |
| 15 | 31.02 | 1.321 (13.21 kGs) | 1775.08 (22.3 kOe) | 0.99 | 696 | 396 |
| 16 | 31.08 | 1.319 (13.19 kGs) | 1775.08 (22.3 kOe) | 0.97 | 703 | 411 |
| 17 | 31.18 | 1.316 (13.16 kGs) | 1783.04 (22.4 kOe) | 0.98 | 696 | 374 |
| 18 | 31.18 | 1.316 (13.16 kGs) | 1791.00 (22.5 kOe) | 0.98 | 655 | 396 |
| 19 | 31.16 | 1.317 (13.17 kGs) | 1775.08 (22.3 kOe) | 0.98 | 694 | 387 |
| 20 | 31.10 | 1.321 (13.21 kGs) | 1775.08 (22.3 kOe) | 0.98 | 668 | 366 |
| max | 31.20 | 1.323 (13.23 kGs) | 1791.00 (22.5 kOe) | 0.99 | 705 | 412 |
| min | 30.97 | 1.316 (13.16 kGs) | 1767.12 (22.2 kOe) | 0.95 | 649 | 354 |
| max-min | 0.23 | 0.007 (0.07 kGs) | 23.88 (0.3 kOe) | 0.04 | 56 | 58 |
| ave | 31.10 | 1.319 (13.19 kGs) | 1777.07 (22.3 kOe) | 0.97 | 680 | 383 |
| δ | 0.09 | 0.02 | 0.10 | 0.01 | | |

According to the data in table 1, the maximum total rare earth element content (TRE) is 31.2 wt.%, the minimum value is 30.97 wt.%, the maximum deviation is 0.23 wt.%, the standard deviation is 0.09. And the maximum value of Br is 1.323 T (13.23 kGs), the minimum value is 1.316 T (13.16 kGs), the maximum deviation of Br is 0.007 T (0.07 kGs), the standard deviation is 0.02. The maximum value of Hcj is 1791,00 kA/m (22.5kOe), the minimum is 1767.12 kA/m (22.2 kOe), the average value is 1777.07 kA/m (22.3kOe), the maximum deviation is 23.88 kA/m (0.3 kOe), the standard deviation is 0.10. The average squareness (Hk/Hcj) value is 0.97. The average value of O element content is 680 ppm, and the average value of N element content is 383 ppm.

### IMPLEMENTING EXAMPLE 2

The target size of product is: 10.0 mm (non-orientation surface) * 6.5 mm (orientation surface) * 8.0 mm (pressing surface), the non-orientation surface and orientation surface were processed into a corresponding size of the finished product by using the special device of the present invention in the green state. The pressing surface were processed after annealing. Specific steps are as follows:

The magnetic powder with an average particle size of X50=4.0 µm was pressed into a green compact under 2.0T magnetic field, and then pressed by isostatic pressing at 400 MPa. The density of green compact after isostatic pressing was about 5.5 g/cm³, and the green compact size was 75.7 mm (non-orientation surface) *33.9mm (orientation surface) * 43.2mm (pressing surface). Green compact weights 609.7g. The magnetic powder composition is PrNd 31.10 wt.%, Dy 1.50 wt.%, B 0.95 wt.%, Co 1.05 wt.%, Al 0.51 wt.%, Cu 0.15 wt.%, Ga 0.12 wt.%, Ti 0.11 wt.% .The balance is Fe and inevitable impurity elements. At first, the wire groove plate with the groove width of 10.8 mm was selected, and the green compact was fastened by adjusting the bolt. A limit baffle with a slot spacing of 10.8mm is selected on the cutting tooling, and the diameter of the cutting wire used is 0.3mm. Start cutting the green compact along the non-orientation surface after the device is assembled. Each green compact is cut into 7 pieces with size of 10.5mm (non-orientation surface)*33.9mm (orientation surface)*43.2mm (pressing surface). And then wire groove plate with the groove width of 8.4 mm and a limit baffle with a slot spacing of 8.4 mm were used to cut the green compacts above along the orientation surface. At last, 28 pieces of green compacts were obtained with the size of 10.5mm (non-orientation surface)*8.1mm (orientation surface)*43.2mm (pressing surface). The above operation was carried out in argon atmosphere. The magnetic powder produced by the cutting process can be simply collected and then subjected to secondary molding. The cut blank is sintered in a vacuum furnace. The sintering temperature was 1040°C, and the temperature was kept for 7 hours. And then the sintered blank was annealed. The first-stage annealing temperature is 900°C, the temperature is kept for 3 hours, the second-stage aging temperature is 600°C, and the temperature is kept for 3 hours. The degree of vacuum during sintering and annealing was less than 5 x 10⁻¹ Pa. The annealing finished blank is subjected to conventional machining. The size was cut into 8.0mm on the pressing surface. And the orientation surface and the non-orientation surface are polished by conventional equipment. Each green compact finally obtained 140 pieces of finished products having a size of 10.0 mm * 6.5 mm * 8.0 mm. During the green machining process, each isostatic green compact produces 36.2g of magnetic powder, which can be directly pressed into a green compact after simple recycling. 25.8g of hard-to-recycle waste powder is produced during the sintering process and annealing process and traditional machining process. Total weight of the finished product is 546.0g, and the comprehensive utilization rate of the magnetic powder is 95.3%. Twenty pieces of products are selected randomly for analyzing. Total rare earth element content (TRE) and magnetic properties are listed in table 2.

**Table 2: TRE and magnetic properties distribution of example 2**

| sample | TRE(wt.%) | Br (T) | Hcj (kA/m) | Hk/Hcj | O (ppm) | N (ppm) |
|---|---|---|---|---|---|---|
| 1 | 31.03 | 1.322 (13.22 kGs) | 1775.08 (22.3 kOe) | 0.97 | 691 | 394 |
| 2 | 31.07 | 1.321 (13.21 kGs) | 1783.04 (22.4 kOe) | 0.98 | 694 | 375 |
| 3 | 31.17 | 1.318 (13.18 kGs) | 1783.04 (22.4 kOe) | 0.98 | 686 | 369 |
| 4 | 31.12 | 1.320 (13.20 kGs) | 1783.04 (22.4 kOe) | 0.98 | 687 | 375 |
| 5 | 31.09 | 1.319 (13.19 kGs) | 1775.08 (22.3 kOe) | 0.99 | 722 | 374 |
| 6 | 31.10 | 1.319 (13.19 kGs) | 1783.04 (22.4 kOe) | 0.98 | 657 | 401 |
| 7 | 31.10 | 1.319 (13.19kGs) | 1783.04 (22.4 kOe) | 0.97 | 705 | 415 |
| 8 | 31.04 | 1.321 (13.21 kGs) | 1775.08 (22.3 kOe) | 0.96 | 687 | 394 |
| 9 | 31.04 | 1.321 (13.21 kGs) | 1783.04 (22.4 kOe) | 0.95 | 725 | 388 |
| 10 | 31.05 | 1.321 (13.21 kGs) | 1775.08 (22.3 kOe) | 0.98 | 697 | 407 |
| 11 | 31.16 | 1.318 (13.18 kGs) | 1791.00 (22.5 kOe) | 0.97 | 675 | 420 |
| 12 | 31.07 | 1.321 (13.21 kGs) | 1783.04 (22.4 kOe) | 0.96 | 701 | 401 |
| 13 | 31.09 | 1.320 (13.20 kGs) | 1783.04 (22.4 kOe) | 0.97 | 696 | 374 |
| 14 | 31.09 | 1.320 (13.20 kGs) | 1783.04 (22.4 kOe) | 0.98 | 667 | 423 |
| 15 | 31.08 | 1.319 (13.19 kGs) | 1783.04 (22.4 kOe) | 0.99 | 702 | 396 |
| 16 | 31.09 | 1.319 (13.19 kGs) | 1775.08 (22.3 kOe) | 0.97 | 696 | 411 |
| 17 | 31.16 | 1.318 (13.18 kGs) | 1791.00 (22.5 kOe) | 0.98 | 678 | 387 |
| 18 | 31.05 | 1.320 (13.20 kGs) | 1783.04 (22.4 kOe) | 0.98 | 685 | 395 |
| 19 | 31.16 | 1.318 (13.18 kGs) | 1791.00 (22.5 kOe) | 0.98 | 701 | 397 |
| 20 | 31.10 | 1.320 (13.20 kGs) | 1775.08 (22.3 kOe) | 0.98 | 679 | 401 |
| max | 31.17 | 1.322 (13.22 kGs) | 1791.00 (22.5 kOe) | 0.99 | 725 | 423 |
| min | 31.03 | 1.318 (13.18 kGs) | 1775.08 (22.3 kOe) | 0.95 | 657 | 369 |
| max-min | 0.14 | 0.004 (0.04 kGs) | 15.92 (0.2 kOe) | 0.04 | 68 | 54 |
| ave | 31.09 | 1.320 (13.20 kGs) | 1783.04 (22.4 kOe) | 0.97 | 692 | 395 |
| δ | 0.04 | 0.01 | 0.07 | 0.01 | | |

According to the data in Table 2, the maximum total rare earth element content (TRE) is 31.17 wt.%, the minimum value is 31.03 wt.%, the maximum deviation is 0.14 wt.%, the standard deviation is 0.04. And the maximum value of Br is 1.322 T (13.22 kGs), the minimum value is 1.318 T (13.18 kGs), the maximum deviation of Br is 0.004 T (0.04kGs), the standard deviation is 0.01. The maximum value of Hcj is 1791.00 kA/m (22.5 kOe), the minimum is 1775.08 kA/m (22.3 kOe), the average value is 1783.04 kA/m (22.4 kOe), the maximum deviation is 15.92 kA/m (0.2 kOe), the standard deviation is 0.07. The average squareness (Hk/Hcj) value is 0.97. The average value of O element content is 692 ppm, and the average value of N element content is 395 ppm.

### COMPARATIVE EXAMPLE 1

The target size of product is: 10.0 mm (non-orientation surface) * 6.5 mm (orientation surface) * 8.0 mm (pressing surface). No machining is carried out in the green compact state, and the magnet is processed into a finished product size by conventional machining method after annealing.

The magnetic powder with an average particle size of X50=4.0 µm was pressed into a green compact under 2.0T magnetic field, and then pressed by isostatic pressing at 400 MPa. The density of green compact after isostatic pressing was about 5.5 g/cm³, and the green compact size was 75.7 mm (Non-orientation surface) *33.9mm (orientation surface) * 43.2mm (pressing surface). Green compact weights 609.7g. The magnetic powder composition is PrNd 31.10 wt.%, Dy 1.50 wt.%, B 0.95 wt.%, Co 1.05 wt.%, Al 0.51 wt.%, Cu 0.15 wt.%, Ga 0.12 wt.%, Ti 0.11 wt.% .The balance is Fe and inevitable impurity elements. The green compact is sintered in a vacuum furnace. The sintering temperature was 1040°C, and the temperature was kept for 7 hours. And then the sintered blank was annealed. The first-stage annealing temperature is 900°C, the temperature is kept for 3 hours, the second-stage aging temperature is 600°C, and the temperature is kept for 3 hours. The degree of vacuum during sintering and annealing was less than 5 x 10⁻¹ Pa. The annealing finished blank is subjected to conventional machining. Each blank finally obtained 140 pieces of finished products having a size of 10.0 mm * 6.5 mm * 8.0 mm. During the sintering process and annealing process and conventional machining process each blank produces 64.4g of hard-to-recycle waste powder. Total weight of the finished product is 546.0g, and the comprehensive utilization rate of the magnetic powder is 89.6%. Twenty pieces of products are selected randomly for analyzing. Total rare earth element content (TRE) and magnetic properties are listed in table 3.

**Table 3: TRE and magnetic properties distribution of comparative example 1**

| sample | TRE(wt.%) | Br(T) | Hcj(kA/m) | Hk/Hcj | O(ppm) | N (ppm) |
|---|---|---|---|---|---|---|
| 1 | 31.35 | 1.314 (13.14 kGs) | 1775.08 (22.30 kOe) | 0.95 | 672 | 353 |
| 2 | 31.24 | 1.316 (13.16 kGs) | 1767.12 (22.20 kOe) | 0.96 | 675 | 346 |
| 3 | 31.15 | 1.318 (13.18 kGs) | 1743.24 (21.90 kOe) | 0.96 | 664 | 348 |
| 4 | 31.02 | 1.323 (13.23 kGs) | 1735.28 (21.80 kOe) | 0.96 | 684 | 389 |
| 5 | 31.03 | 1.321 (13.21 kGs) | 1743.24 (21.90 kOe) | 0.97 | 695 | 355 |
| 6 | 31.24 | 1.316 (13.16 kGs) | 1767.12 (22.20 kOe) | 0.96 | 678 | 396 |
| 7 | 30.76 | 1.326 (13.26 kGs) | 1727.32 (21.70 kOe) | 0.95 | 632 | 347 |
| 8 | 30.88 | 1.324 (13.24 kGs) | 1735.28 (21.80 kOe) | 0.94 | 667 | 384 |
| 9 | 30.91 | 1.323 (13.23 kGs) | 1735.28 (21.80 kOe) | 0.95 | 668 | 386 |
| 10 | 31.39 | 1.311 (13.11 kGs) | 1775.08 (22.30 kOe) | 0.96 | 634 | 359 |
| 11 | 30.92 | 1.324 (13.24 kGs) | 1727.32 (21.70 kOe) | 0.95 | 647 | 334 |
| 12 | 30.85 | 1.325 (13.25 | 1735.28 (21.80 kOe) | 0.94 | 678 | 364 |
| | | kGs) | | | | |
| 13 | 31.01 | 1.323 (13.23 kGs) | 1743.24 (21.90 kOe) | 0.95 | 632 | 361 |
| 14 | 31.12 | 1.319 (13.19 kGs) | 1751.20 (22.00 kOe) | 0.96 | 657 | 375 |
| 15 | 31.05 | 1.322 (13.22 kGs) | 1743.24 (21.90 kOe) | 0.97 | 679 | 376 |
| 16 | 30.88 | 1.325 (13.25 kGs) | 1735.28 (21.80 kOe) | 0.95 | 643 | 347 |
| 17 | 30.82 | 1.325 (13.25 kGs) | 1735.28 (21.80 kOe) | 0.96 | 656 | 356 |
| 18 | 31.26 | 1.318 (13.18 kGs) | 1759.16 (22.10 kOe) | 0.96 | 634 | 401 |
| 19 | 31.35 | 1.313 (13.13 kGs) | 1775.08 (22.30 kOe) | 0.96 | 674 | 374 |
| 20 | 31.42 | 1.310 (13.10 kGs) | 1783.04 (22.40 kOe) | 0.96 | 687 | 368 |
| max | 31.42 | 1.326 (13.26 kGs) | 1783.04 (22.40 kOe) | 0.97 | 695 | 401 |
| min | 30.76 | 1.310 (13.10 kGs) | 1727.32 (21.70 kOe) | 0.94 | 632 | 334 |
| max-min | 0.66 | 0.016 (0.16 kGs) | 55.72 (0.70 kOe) | 0.03 | 63 | 67 |
| ave | 31.08 | 1.320 (13.20 kGs) | 1743.24 (21.9 kOe) | 0.96 | 663 | 366 |
| δ | 0.21 | 0.05 | 0.23 | 0.01 | | |

According to the data in Table 3, the maximum total rare earth element content (TRE) is 31.42 wt.%, the minimum value is 30.76 wt.%, the maximum deviation is 0.66 wt.%, the standard deviation is 0.21. And the maximum value of Br is 1.326 T (13.26 kGs), the minimum value is 1.310 T (13.10kGs), the maximum deviation of Br is 0.016 T (0.16kGs), the standard deviation is 0.05. The maximum value of Hcj is 1783.04 kA/m (22.4kOe), the minimum is 1727.32 kA/m (21.7kOe), the average value is 1749.61 kA/m (21.9kOe), the maximum deviation is 55.72 kA/m (0.7kOe), the standard deviation is 0.23. The average squareness (Hk/Hcj) value is 0.96. The average value of O element content is 663 ppm, and the average value of N element content is 366 ppm.

### COMPARATIVE EXAMPLE 2

The target size of product is: 10.0 mm (non-orientation surface) * 6.5 mm (orientation surface) * 8.0 mm (pressing surface), the non-orientation surface and orientation surface and pressing surface were all processed into a corresponding size of the finished product by using the special device of the present invention in the green state. Specific steps are as follows:
The magnetic powder with an average particle size of X50=4.0 µm was pressed into a green compact under 2.0T magnetic field, and then pressed by isostatic pressing at 400 MPa. The density of green compact after isostatic pressing was about 5.5 g/cm³, and the green compact size was 75.7 mm (Non-orientation surface) *33.9mm (orientation surface) * 43.2mm (pressing surface). Green compact weights 609.7g. The magnetic powder composition is PrNd 31.10 wt.%, Dy 1.50 wt.%, B 0.95 wt.%, Co 1.05 wt.%, Al 0.51 wt.%, Cu 0.15 wt.%, Ga 0.12 wt.%, Ti 0.11 wt.% .The balance is Fe and inevitable impurity elements. Using the special device of the present invention to process the green compact. Firstly, the wire groove plate with the groove width of 10.8 mm was selected, and the green compact was fastened by adjusting the bolt. A limit baffle with a slot spacing of 10.8mm is selected on the cutting tooling, and the diameter of the cutting wire used is 0.3mm. Start cutting the green compact along the non-orientation surface after the device is assembled.

Each green compact is cut into 7 pieces with size of 10.5mm (non-orientation surface)*33.9mm (orientation surface)*43.2mm (pressing surface). Secondly, wire groove plate with the groove width of 8.4 mm and a limit baffle with a slot spacing of 8.4 mm were used to cut the green compacts above along the orientation surface. 28 pieces of green compacts were obtained with the size of 10.5mm (non-orientation surface)*8.1mm (orientation surface)*43.2mm (pressing surface). Thirdly, wire groove plate with the groove width of 8.6 mm and a limit baffle with a slot spacing of 8.6 mm were used to cut the green compact above along the pressing surface. At last, 140 pieces of green compacts were obtained with the size of 10.5mm (non-orientation surface)*8.1mm (orientation surface)*8.3mm (pressing surface).The above operation was carried out in argon atmosphere. The magnetic powder produced by the cutting process can be simply collected and then subjected to secondary molding. The cut green compact was sintered in a vacuum furnace. The sintering temperature was 1040°C, and the temperature was kept for 7 hours. And then the sintered blank was annealed. The first-stage annealing temperature is 900°C, the temperature is kept for 3 hours, the second-stage annealing temperature is 600°C, and the temperature is kept for 3 hours. The degree of vacuum during sintering and annealing was less than 5 x 10⁻¹ Pa. The annealing finished blank is subjected to conventional machining, a simple mechanical grinding and polishing was performed on three surfaces. Each of the isostatically pressed blanks finally obtains 140 finished products having a size of 10.0 mm*6.5 mm*8.0 mm. During the green machining process, each isostatic green compact produces 50.8g of magnetic powder, which can be directly pressed into a green compact after simple recycling. 12.0g of hard-to-recycle waste powder was produced during the sintering process and annealing process and traditional machining process. Total weight of the finished product is 546.0g, and the comprehensive utilization rate of the magnetic powder is 97.7%. Twenty pieces of products are selected randomly for analyzing. Total rare earth element content (TRE) and magnetic properties are listed in table 4.

**Table 4: TRE and magnetic properties distribution of comparative example 2**

| sample | TRE(wt.%) | Br(T) | Hcj(kA/m) | Hk/Hcj | O (ppm) | N (ppm) |
|---|---|---|---|---|---|---|
| 1 | 31.09 | 1.320 (13.20 kGs) | 1767.12 (22.2 kOe) | 0.95 | 731 | 453 |
| 2 | 31.10 | 1.316 (13.16 kGs) | 1759.16 (22.1 kOe) | 0.96 | 742 | 466 |
| 3 | 31.05 | 1.318 (13.18 kGs) | 1751.20 (22.0 kOe) | 0.94 | 725 | 457 |
| 4 | 31.16 | 1.320 (13.20 kGs) | 1767.12 (22.2 kOe) | 0.95 | 718 | 447 |
| 5 | 31.10 | 1.319 (13.19 kGs) | 1759.16 (22.1 kOe) | 0.96 | 719 | 453 |
| 6 | 31.10 | 1.319 (13.19 kGs) | 1767.12 (22.2 kOe) | 0.96 | 713 | 467 |
| 7 | 31.07 | 1.314 (13.14 kGs) | 1743.24 (21.9 kOe) | 0.96 | 722 | 446 |
| 8 | 31.07 | 1.317 (13.17 kGs) | 1735.28 (21.8 kOe) | 0.96 | 676 | 495 |
| 9 | 31.09 | 1.317 (13.17 kGs) | 1751.20 (22.0 kOe) | 0.95 | 759 | 446 |
| 10 | 31.16 | 1.317 (13.17 kGs) | 1767.12 (22.2 kOe) | 0.97 | 753 | 445 |
| 11 | 31.10 | 1.318 (13.18 kGs) | 1751.20 (22.0 kOe) | 0.96 | 734 | 426 |
| 12 | 31.07 | 1.319 (13.19 kGs) | 1743.24 (21.9 kOe) | 0.96 | 731 | 434 |
| 13 | 31.17 | 1.320 (13.20 kGs) | 1775.08 (22.3 kOe) | 0.97 | 726 | 485 |
| 14 | 31.09 | 1.320 (13.20 kGs) | 1735.28 (21.8 kOe) | 0.96 | 725 | 494 |
| 15 | 31.08 | 1.319 (13.19 kGs) | 1751.20 (22.0 kOe) | 0.96 | 677 | 501 |
| 16 | 31.09 | 1.319 (13.19 kGs) | 1759.16 (22.1 kOe) | 0.96 | 724 | 466 |
| 17 | 31.16 | 1.318 (13.18 kGs) | 1767.12 (22.2 kOe) | 0.94 | 711 | 431 |
| 18 | 31.05 | 1.321 (13.21 kGs) | 1727.32 (21.7 kOe) | 0.94 | 724 | 436 |
| 19 | 31.16 | 1.318 (13.18 kGs) | 1775.08 (22.3 kOe) | 0.95 | 675 | 435 |
| 20 | 31.10 | 1.320 (13.20 kGs) | 1751.20 (22.0 kOe) | 0.96 | 687 | 446 |
| max | 31.17 | 1.321 (13.21 kGs) | 1775.08 (22.3 kOe) | 0.97 | 759 | 501 |
| min | 31.05 | 1.314 (13.14 kGs) | 1727.32 (21.7 kOe) | 0.94 | 675 | 426 |
| max-min | 0.12 | 0.007 (0.07 kGs) | 47.76 (0.6 kOe) | 0.03 | 84 | 75 |
| ave | 31.10 | 1.318 (13.18 kGs) | 1759.16 (22.1 kOe) | 0.96 | 719 | 456 |
| δ | 0.04 | 0.02 | 0.17 | 0.01 | | |

According to the data in table 4, the maximum total rare earth element content (TRE) is 31.17 wt.%, the minimum value is 31.05 wt.%, the maximum deviation is 0.12 wt.%, the standard deviation is 0.04. And the maximum value of Br is 1.321 T (13.21 kGs), the minimum value is 1.314 T (13.14 kGs), the maximum deviation of Br is 0.007 T (0.07 kGs), the standard deviation is 0.02. The maximum value of Hcj is 1775.08 kA/m (22.3 kOe), the minimum is 1727.32 kA/m (21.7 kOe), the average value is 1759.16 kA/m (22.1 kOe), the maximum deviation is 47.76 kA/m (0.6 kOe), the standard deviation is 0.17. The average squareness (Hk/Hcj) value is 0.96. The average value of O element content is 719 ppm, and the average value of N element content is 456 ppm.

Comparing the results of Example 1, Example 2 and Comparative Example 1, for the sintered NdFeB product prepared by the special device and method of the present invention, maximum deviation and standard deviation value of the total rare earth element and Br and Hcj all become smaller, which means the product uniformity is improved. And the value of Hcj is increased by 0.32∼0.42kOe. At the same time, a part of the magnetic powder generated during the machining can be recycled and reused in a simple manner, which reduces the proportion of the difficult-to-recover magnetic powder generated by the conventional mechanical machining method. And the comprehensive utilization ratio of the magnetic powder is increased from 89.6% to 91.7 to 95.3%.

Comparing the results of example 1, example 2 and comparative example 2, green compact in comparative example 2 was completely processed into corresponding size of product in three surfaces before sintering, which makes the component and Br deviation reduced. But the improvement is not obvious. What's more, the method of comparative example 2 further increases the specific surface area, which causes the green compact to be more easily oxidized and nitride during cutting and sintering process. Then the Hcj gets lower because of higher N and O impurities in the final product. It can be seen that in order to improve the uniformity and magnetic properties, cutting one or two surface of the green compact will play a better role.

## Claims

1. A method of preparing a sintered NdFeB magnet, said method comprising the steps of:
a) pressing magnetic powders into a green compact under a magnetic field and then demagnetization;
b) isostatic pressing the green compact;
c) fixing the green compact on a special device comprising:
a reciprocating cutting mechanism (A), a cutting tooling (B), a green compact fixed tooling (C) and a reciprocating lifting mechanism (D), wherein
the reciprocating cutting mechanism (A) is connected to the cutting tooling (B), the reciprocating lifting mechanism (D) is connected to the green compact fixed tooling (C),
the reciprocating cutting mechanism (A) is adapted for reciprocating in a horizontal direction, and the reciprocating lifting mechanism (D) is adapted for realizing a reciprocating lifting in a vertical direction;
the green compact fixed tooling (C) comprises a pair of trunking plates (1), a pair of limit guiding plates (2), guiding pins (3), adjusting bolts (4) and a base (5), wherein the pair of trunking plates (1) is mounted on opposite sides of the base (5), the pair of limit guiding plates (2) is mounted to the end of the trunking plates (1), and the limit guiding plates (2) are provided with the guiding pins (3) and adjusting bolts (4); and
the cutting tooling (B) comprises a pair of wire fixing boards (6), cutting wires (7), adjusting screws (8), and a fixing plate (9), wherein the pair of wire fixing boards (6) is mounted on the fixing plate (9) and the cutting wires (9) are tensioned by means of the adjusting screws (8) between the the pair of wire fixing boards (6),
and then machining the green compact into a finished shape and corresponding size on one or two surfaces among an orientation surface, non-orientation surface and pressing surface;
d) sintering and annealing the machined green compact; and
e) machining the obtained blank into a finished product.

2. The method of claim 1, wherein in step b) of isostatic pressing the pressure is between 150MPa to 400MPa.

3. The method of claim 1 or 2, wherein the density of green compact after isostatic pressing is between 4.5-5.5g/cm³.

4. The method of any of the preceding claims, wherein in step c) the orientation surface refers to the surface parallel to the orientation magnetic field and not in contact with an indenter during the pressing process;
the pressing surface refers to the plane in contact with the indenter during the pressing process;
the non-orientation surface refers to the plane perpendicular to the orientation surface and the pressing surface; and
the corresponding size of the finished product refers to the size of the finished product multiplied by the shrinkage rate of the sintering process.

5. The method of claim 1, wherein step c) of machining the machining green compact is operated in the atmosphere of nitrogen or rare gas.

6. The method of any of the preceding claims, wherein step d) of sintering and annealing is performed under vacuum of below 5×10⁻¹Pa, a sintering temperature is between 980°C to 1040°C, and an annealing temperature is between 480°C to 600°C.

7. The method of any of the preceding claims, wherein step e) of machining the blank refers to processing
surfaces that have not been processed in step c) of machining the green compact.

## Patentansprüche

1. Verfahren zur Vorbereitung eines gesinterten NdFeB-Magneten, wobei das Verfahren die Schritte umfasst:
a) Pressen von Magnetpulver in einen grünen Pressling unter einem Magnetfeld und dann Entmagnetisieren;
b) isostatisches Pressen des grünen Presslings;
c) Befestigen des grünen Presslings auf einem speziellen Gerät, umfassend:
einen gegenseitigen Schnittmechanismus (A), ein Schneidwerkzeug (B), ein befestigtes Werkzeug (C) für einen grünen Pressling und einen pendelnden Hebemechanismus (D), wobei der pendelnde Schneidmechanismus (A) an das Schneidwerkzeug (B) angeschlossen ist, wobei der pendelnde Hebemechanismus (D) an das befestigte Werkzeug (C) für einen grünen Pressling angeschlossen ist, der pendelnde Schneidmechanismus (A) zum Pendeln in einer horizontalen Richtung geeignet ist und der pendelnde Hebemechanismus (D) zum Realisieren eines pendelnden Hebens in einer vertikalen Richtung geeignet ist;
das befestigte Werkzeug (C) des grünen Presslings umfasst ein Paar von Rumpfplatten (1), ein Paar eingrenzender Führungsplatten (2), Führungsstifte (3), Einstellbolzen (4) und eine Basis (5), wobei das Paar Rumpfplatten (1) auf gegenüberliegenden Seiten der Basis (5) montiert ist, wobei das Paar eingrenzender Führungsplatten (2) am Ende der Rumpfplatten (1) montiert ist und die eingrenzenden Führungsplatten (2) mit den Führungsstiften (3) und Einstellbolzen (4) bereitgestellt sind; und
das Schneidwerkzeug (B) umfasst ein Paar Drahtbefestigungs-Tafeln (6), Schneiddrähte (7), Einstellschrauben (8) und eine Befestigungsplatte (9),
wobei das Paar Drahtbefestigungs-Tafeln (6) auf der Befestigungsplatte (9) montiert ist und die Schneiddrähte (9) mittels der Einstellschrauben (8) zwischen dem Paar Drahtbefestigungs-Tafeln (6) gespannt sind,
und dann Bearbeiten des grünen Presslings in eine Endform und entsprechende Größe auf einer oder zwei Fläche(n) aus einer Ausrichtungsfläche, einer Nicht-Ausrichtungsfläche und einer Druckfläche;
d) Sintern und Glühen des bearbeiteten grünen Presslings; und
e) Bearbeiten des erhaltenen Rohlings in ein Endprodukt.

2. Verfahren nach Anspruch 1, wobei in Schritt b) ein isostatisches Pressen der Druck zwischen 150 MPa und 400 MPa liegt.

3. Verfahren nach Anspruch 1 oder 2, wobei die Dichte des grünen Presslings nach dem isostatischen Pressen zwischen 4,5 und 5,5 g/cm³ liegt.

4. Verfahren nach irgendeinem der voranstehenden Ansprüche, wobei sich in Schritt c) die Ausrichtungsfläche auf die Fläche parallel zu dem Orientierungs-Magnetfeld bezieht und während des Pressprozesses nicht mit einem Eindruckkörper in Kontakt ist;
die Druckfläche bezieht sich auf die Ebene, die während des Pressprozesses mit dem Eindruckkörper in Kontakt ist;
die Nicht-Ausrichtungsfläche bezieht sich auf die Ebene, die zu der Ausrichtungsfläche und der Druckfläche lotrecht ist; und
die entsprechende Größe des Endprodukts bezieht sich auf das Endprodukt, multipliziert mit der Schwindungsrate des Sinterprozesses.

5. Verfahren nach Anspruch 1, wobei Schritt c) des Bearbeitens die Bearbeitung des grünen Presslings in einer Atmosphäre aus Stickstoff oder Edelgas durchgeführt wird.

6. Verfahren nach irgendeinem der voranstehenden Ansprüche, wobei Schritt d) des Sinterns und Glühens unter Vakuum von weniger als 5 x 10⁻¹ Pa durchgeführt wird, eine Sintertemperatur zwischen 980°C und 1040 °C beträgt und eine Glühtemperatur zwischen 480°C und 600 °C beträgt.

7. Verfahren nach irgendeinem der voranstehenden Ansprüche, wobei Schritt e) des Bearbeitens des Rohlings sich auf das Verarbeiten von Flächen bezieht, die in Schritt c) des Bearbeitens des grünen Presslings nicht verarbeitet wurden.

## Revendications

1. Procédé de préparation d'un aimant NdFeB fritté, ledit procédé comprenant les étapes de:
a) pressage des poudres magnétiques en un compact vert sous un champ magnétique puis démagnétisation;
b) pressage isostatique du compact vert;
c) fixation du compact vert sur un dispositif spécial comprenant :
un mécanisme de coupe à mouvement alternatif (A), un outil de coupe (B), un outillage fixe de compact vert (C) et un mécanisme de levage à mouvement alternatif (D), dans lequel le mécanisme de coupe à mouvement alternatif (A) est raccordé à l'outillage de coupe (B), le mécanisme de levage alternatif (D) est raccordé à l'outillage fixe de compact vert (C),
le mécanisme de coupe alternatif (A) est adapté pour un mouvement alternatif dans une direction horizontale, et le mécanisme de levage alternatif (D) est adapté pour réaliser un levage alternatif dans une direction verticale;
l'outillage fixe de compact vert (C) comprend une paire de plaques de goulotte (1), une paire de plaques de guidage de limite (2), des goupilles de guidage (3), des boulons de réglage (4) et une base (5), dans lequel la paire de plaques de goulotte (1) est montée sur les côtés opposés de la base (5), la paire de plaques de guidage de limite (2) est montée à l'extrémité des plaques de goulotte (1) et les plaques de guidage de limite (2) sont pourvues des broches de guidage (3) et les boulons de réglage (4); et
l'outillage de coupe (B) comprend une paire de plaques de fixation de fil (6), des fils de coupe (7), des vis de réglage (8) et une plaque de fixation (9), dans lequel la paire de plaques de fixation de fil (6) est montée sur la plaque de fixation (9) et les fils de coupe (9) sont tendus au moyen des vis de réglage (8) entre la paire de plaques de fixation de fil (6),
puis usinage du compact vert en une forme finie et de la taille correspondante sur une ou deux surfaces parmi une surface d'orientation, une surface sans orientation et une surface de pression;
d) frittage et recuit du compact vert usiné; et
e) usinage de l'ébauche obtenue en un produit fini.

2. Procédé selon la revendication 1, dans lequel à l'étape b) de pressage isostatique la pression est comprise entre 150MPa et 400MPa.

3. Procédé selon la revendication 1 ou 2, dans lequel la densité du compact vert après pressage isostatique est comprise entre 4,5 et 5,5 g/cm³.

4. Procédé selon une quelconque des revendications précédentes, dans lequel à l'étape c) la surface d'orientation se réfère à la surface parallèle au champ magnétique d'orientation et non en contact avec un pénétrateur pendant le processus de pressage;
la surface de pressage se réfère au plan en contact avec le pénétrateur pendant le processus de pressage; la surface de non-orientation fait référence au plan perpendiculaire à la surface d'orientation et à la surface de pression; et
la taille correspondante du produit fini se réfère à la taille du produit fini multipliée par le taux de retrait du processus de frittage.

5. Procédé selon la revendication 1, dans lequel l'étape c) d'usinage du compact vert d'usinage est mise en œuvre sous atmosphère d'azote ou de gaz rare.

6. Procédé selon une quelconque des revendications précédentes, dans lequel l'étape d) de frittage et de recuit est effectuée sous un vide inférieur à 5×10⁻¹ Pa, une température de frittage est comprise entre 980°C et 1040°C, et une température de recuit est comprise entre 480°C à 600°C.

7. Procédé selon une quelconque des revendications précédentes, dans lequel l'étape e) d'usinage de l'ébauche se réfère à des surfaces de traitement qui n'ont pas été traitées à l'étape c) d'usinage du compact vert.
